

Patented Apr. 3, 1923.

1,450,600

## UNITED STATES PATENT OFFICE.

AUGUST LENDLE, OF FOREST HILLS, NEW YORK, ASSIGNOR TO KUTTROFF PICKHARDT & CO., INC., OF NEW YORK, N. Y., A CORPORATION OF NEW YORK.

### PAPER MADE FROM KAPOK FIBER.

No Drawing.

Application filed September 9, 1920. Serial No. 409,245.

To all whom it may concern:

Be it known that I, AUGUST LENDLE, a citizen of the United States, residing at Forest Hills, county of Queens, and State of New York, have invented new and useful Improvements in Paper Made from Kapok Fiber, of which the following is a specification.

My invention consists of a new process of manufacturing paper and comprises the use of a new basic material in the manufacture of paper.

Paper made by my process is of a silky textile-like texture and appearance and is particularly adapted for use as a highly finished wall paper and is adaptable also for covering boxes, etc. Heretofore in order to obtain the silky-like effect in paper it has been necessary to sprinkle the paper with silk which process is very laborious and expensive.

The invention consists in using as the essential ground work of the paper a substance commercially known as kapok.

The kapok is a fiber found in tropical countries, and is now being used in the manufacture of mattresses, pillows, life belts, etc. If ground in beaters such as are commonly used in paper mills, it can be cut up so as to make it practical for use in the manufacture of papers. It may be used by itself alone or in connection with other fibers, such as ground wood, sulphite, saw dust, rag, jute, etc.

The following are suitable examples of the process, but my invention is not limited thereto.

#### Example I.

A kapok fiber is put in a beater and then colored with suitable dyestuffs at ordinary

or raised temperature then beaten for a sufficient time to make the fiber flow on a paper machine. The resulting paper has a distinct silky appearance entirely different from any paper heretofore known.

#### Example II.

Saw dust is colored with suitable dyestuffs then mixed with kapok previously beaten and dyed as set forth in example I. The resulting paper shows a distinct silky effect and appearance, not known heretofore.

#### Example III.

Saw dust is colored with suitable dyestuffs and mixed with undyed kapok, but previously sufficiently beaten.

#### Example IV.

Kapok fiber is put in a beater and then colored with suitable dyestuffs, then beaten sufficiently to which is then added uncolored saw dust.

I claim:—

1. As a new article of manufacture a paper made from kapok fiber.
2. As a new article of manufacture a paper made from kapok, and other substances.
3. As a new article of manufacture a paper made from kapok, and vegetable substances.
4. As a new article of manufacture a paper made from kapok, and ground wood.

In testimony whereof I have hereunto set my hand in the presence of two subscribing witnesses.

AUGUST LENDLE.

Witnesses:

Wm. P. PICKHARDT,  
H. STOLZE.